

Sept. 25, 1923.

J. F. L. BAKER

1,468,692

METHOD OF MAKING BOILER HEADERS

Filed April 25, 1921



*John F. L. Baker*  
INVENTOR  
BY *Geo. B. Wilcox*

ATTORNEY

## UNITED STATES PATENT OFFICE.

JOHN F. L. BAKER, OF SAGINAW, MICHIGAN, ASSIGNEE TO THE WICKES BOILER COMPANY, OF SAGINAW, MICHIGAN, A CORPORATION OF MICHIGAN.

## METHOD OF MAKING BOILER HEADERS.

Application filed April 25, 1921. Serial No. 464,891.

To all whom it may concern:

Be it known that I, JOHN F. L. BAKER, a citizen of the United States, residing at Saginaw, in the county of Saginaw and 5 State of Michigan, have invented certain new and useful Improvements in Methods of Making Boiler Headers; and I do hereby declare the following to be a full, clear, and exact description of the invention, such as 10 will enable others skilled in the art to which it appertains to make and use the same.

This invention relates to headers for water tube boilers and the like and the objects 15 of my improvement are, to simplify and improve the method of making wide headers, that is to say, headers, the front and back plates of which are so far separated as to form a water space, or steam space of considerable width, say, ten inches or wider. 20 My improvement relates more particularly to the method which I employ in forming or fabricating the flanged plates constituting the tube sheets of the header, and to the forming dies by which the method is 25 carried out in practice.

It has heretofore been customary in water tube boiler manufacturing practice to flange the two sheets forming the walls of the header or water leg, and to back one of 30 the heads into the other, riveting or calking the outer edge of the joint so formed.

Formerly the edges of the header plates were bent to form side and end flanges, and the corner produced by the junction of the 35 body of the plate with the side and end flanges was then heated and pressed into shape by one operation of a forming die.

It has, however, been impossible by the 40 above-mentioned operation to produce a satisfactory flanged corner on a heavy plate, say, five-eighths inch thick and having a flange over four inches in depth; because the junction of the flanges at the corners of the plate could not be satisfactorily formed with deeper flanges, on account of the tendency of the surplus material at the corners 45 to fold and crinkle and in some places to stretch and become thin.

The tube sheets of headers having water 50 spaces ten inches or more in width require wide flanges, say, thirteen to fifteen inches deep, and consequently the former method is not adequate for the manufacture of headers having very deep flanges, that are bent to radii of, say, six inches and over.

Such a large-radius flange construction is shown in my Patent 1,408,244.

By my present improved method I produce headers from thick material, say, five-eighths inch or thicker, and flanges to radii 60 of six inches and over, the corners at the junction of the flanges formed with a truly spherical heel, each corner heel representing one-eighth of the surface of a sphere, the radius of which is equal approximately to 65 the distance between the plates of the finished header.

Some of the practical advantages of the long-radius type of flange for boiler headers are set forth in my co-pending application above referred to. My present method of forming the flanged corners without cutting or welding, and while maintaining the normal thickness of metal, is particularly 70 well adapted to the forming of long-radius, 75 deep flanged header plates, because the long-radius flanges can readily be formed at the corners into an integral, long-radius spherical heel, and such a heel utilizes the greatest amount possible of the plate material at the 80 corner, and consequently requires a minimum amount of material to be pressed or flowed to maintain the required uniform thickness.

It is essential in boiler work of this 85 character that the final thickness of the formed or flanged plates shall be uniform. That is to say, the thickness at one point of the spherical corner shall be the same as the thickness at any point on the flange, or any 90 point on the body of the plate. By my improved method I produce flanged and formed header plates of uniform thickness at the flanges and corners and prevent the permanent stretching of the material and the formation of thin spots. I cause the metal while being flanged to flow to those parts which normally would be formed thin and consequently I maintain those parts at 95 the desired thickness.

With the above and certain other objects in view, which will appear later in the specification, my invention consists in the method and means herein described and the equivalents thereof.

My improved method of constructing from thick plates headers having very wide flanges, say, from ten to fifteen inches, and formed with large radii, the junction of the flanges at the corners of the plates being 110

spherical and of uniform thickness, is illustrated in the accompanying drawings, in which Fig. 1 is a fragmentary transverse section through one end of a boiler header, 5 showing a wide flanged tube sheet made in accordance with my improved method.

Fig. 2 is a perspective view of a formed and flanged tube sheet, the position of the metal at the commencement of the corner-forming operation being indicated by dotted lines.

Fig. 3 is a fragmentary plan view showing a corner of a tube sheet trimmed preparatory to flanging, the part removed by 15 trimming being indicated by dotted lines.

Fig. 4 is a fragmentary plan view showing a corner of a flanged tube sheet.

Fig. 5 is a perspective view, showing the corner of a tube sheet as it appears after the 20 side edges of the sheet are flanged, one side edge shown between the dies of a flanging press.

Fig. 6 is a side elevation of a pair of dies with a plate between, the edges of which 25 have been flanged as in Fig. 5, and the projecting corner in place for the second or main corner-forming operation, the die plunger shown in its raised position.

Fig. 7 is a similar view after the die 30 plunger has descended, the plunger in this view being shown in vertical section.

Fig. 8 is a top plan view of the plunger shown in Fig. 7.

Fig. 9 is an elevation of the working face 35 of the die plunger.

Fig. 10 is a horizontal section on the line 10—10 of Fig. 9.

Fig. 11 is a similar section on the line 11—11 of Fig. 9.

40 Fig. 12 is an enlarged fragmentary section through the plate shown in Fig. 7, showing the increased thickness of the edge of the plate at the extremity of the corner after performing the second forming operation indicated in Fig. 7.

Fig. 13 is a side view of the dies used for the third or final flanging step of my method, the plate being shown in the die in the condition in which it was removed from the 50 second flanging step illustrated in Fig. 7, the die plunger of Fig. 13 being in its raised position.

Fig. 14 is a part sectional side elevation of the parts shown in Fig. 13, with the 55 plunger down, completing the formation of the top flange of the header.

In employing my method, I first take a steel plate 1 of proper size and thickness, say, five-eighths inch, trimming each corner 2, 60 to a somewhat circular shape.

The rounded corner is then heated and slightly formed by being bent downward in the roughing die illustrated in Fig. 7.

The side edge 3 and edge 4 of the plate 65 are then successively heated and flanged in.

a suitable press 5, as indicated in Fig. 5, to produce a flange of approximately six inch or greater radius and of any desired depth up to, say, fifteen inches.

After the edges 3 and 4 of the plate have 70 been flanged, each corner shows an outwardly projecting scoop-shaped or hood like part 6, as shown in Figs. 5 and 6, and it is from these scoop-shaped corner projections that the final large-radius spherical heel or 75 corner of the header is afterward formed.

The next step is to re-heat the scoop-shaped corner 6 and to place the hot plate on the forming die block 7 of the roughing die, where the heel or spherical part 8 of 80 the corner is formed, leaving that part 9 of the plate, which is to form the upright corner flange, projecting outwardly and downwardly from the plane of the plate 1, at an angle of approximately sixty degrees, 85 as indicated in Fig. 12. Examination of the plate at the outer edge 10 of a corner so formed discloses that the outwardly projecting part of the plate is thicker by approximately one-eighth inch than the thickness of 90 the heel 8, or of the body 1, of the plate. If the plate is five-eighths inch thick, it will be found after the heel-forming operation of Fig. 7, that the outer edge 10 of the plate, 95 at the corner, is approximately three-fourths inch thick, and that this thickness gradually decreases from the extreme edge to the normal thickness of about five-eighths inch at the spherical part or heel 8, showing that the 100 heated surplus material in the plate at the corner has been caused, by the pressure of the heel-forming die, to flow into the outer part 10 of the corner lip. By the term surplus material, I mean the amount of metal which is in excess of the amount required to 105 form a spherical corner and flange equal in thickness to the thickness of the plate. This surplus is present because less metal is required to be present in the finished spherical heel and flange than is present in the 110 corner portion of the flat trimmed plate.

For many years it has been demonstrated in practice that when the complete corner-forming operation is attempted to be accomplished by a single operation of a forming die, crinkling, stretching, or otherwise distorting the metal at the corner can only be avoided if shallow flanges are formed. Such crinkling is inevitable with a single-operation die when deep flanges are formed, 115 because a single die is incapable of both forming the corner and forcing metal to flow into proper position in the heel and flanges.

I, therefore, form the heel 8 and only partially form the flange-walls 3, 4 of the corner in the die operation just described, and employ a further or third step to complete the corner-forming operation. In this third 120 step, I reheat the corner of the plate and 125

place the partly formed corner under a vertically movable finishing die 11, of partly-cylindrical shape, as in Figs. 13 and 14. This die 11 completes the straightening or bending to ninety degrees of the flange, Fig. 12, as it was left by the heel-forming die 7 at an angle of approximately sixty degrees from the plane of the plate. This finishing die 11 is so backed or supported and held at a fixed distance from the die block and plate by the guide 12 that it can not spring. It, therefore, produces a finished flange of correct and uniform thickness, say, five-eighths inch, and distributes the thick metal between edge 10 and the heel 8 left by the previous operation, in such manner that part of the metal will flow laterally as indicated by the arrow in Fig. 14 to make up the desired thickness of the side walls of the flanges 3 and 4 and the other part of the surplus metal will flow downward, and will form a slightly projecting lip 13, which lip is found to be of considerably greater thickness than the thickness of the plate. The edge of this lip can later be trimmed off flush with the side flanges 3 and 4.

Notwithstanding the fact that former methods which I have herein previously described, can be depended upon to produce satisfactory flanged headers having flanges of not over, say, four inches in depth, it is a demonstrated fact that for headers requiring the use of heavy flanges of relatively great depth, say, from four to fifteen inches, the former flanging methods are not practicable on account of the amount of material in the plate at the corner. My present improvement, however, entirely overcomes the difficulties of the former method and renders it perfectly feasible to properly form flanged corners of great depth.

Having thus described my invention, what I claim and desire to secure by Letters Patent is:

1. The herein described method of forming deep-flanged headers comprising trimming the corners of the header plate, to approximately circular form, heating a corner and pressing it to bend the edges at the corner slightly downwardly, heating the side edges of the plate and flanging them to a large radius and thereby forming an elongated scoop-shaped projection at each corner, re-heating and pressing said projection to form a practically spherical heel of the same radius as the flange radius, bend-

ing the projecting part of the scoop-shaped corner downwardly to an angle of approximately sixty degrees from the plane of the plate, re-heating the corner and pressing said projection into a position at right angles to the plane of the plate while simultaneously forcing a portion of the surplus metal of said projection to flow laterally into the flanges, to thereby restore said parts to uniform thickness.

2. The herein described method of forming deep flanged headers comprising trimming corners of the header plate to approximately circular form, heating the side edges of the plate and flanging them to a large radius, thereby forming an elongated scoop-shaped projection at each corner, re-heating and pressing said projection to form a spherical heel of the same radius as the flange radius, re-heating the corner and pressing said projection into a position at right angle to the plane of the plate while simultaneously forcing a portion of the surplus metal of said projection to flow laterally into the flanges to thereby restore said parts to uniform thickness.

3. The herein described method of forming deep flanged headers comprising trimming the corners of the header plate to approximately circular form, bending the side edges of the plate to a large radius, thereby forming an elongated scoop-shaped projection at each corner, heating and pressing said projection to form an approximately spherical heel of approximately the same radius as the flange radius, re-heating the corner and pressing said projection into a position at right angle to the plane of the plate.

4. The herein described method of forming deep flanged headers comprising trimming the corners of the header plate to approximately circular form, bending the side edges of the plate to a large radius, thereby forming an elongated scoop-shaped projection at each corner, heating and pressing said projection to form an approximately spherical heel of approximately the same radius as the flange radius, re-heating the corner and pressing said projection into a position at right angle to the plane of the plate while simultaneously forcing a portion of the surplus metal of said projection to flow into the flanges.

In testimony whereof, I affix my signature.

JOHN F. L. BAKER.